

# UNITED STATES PATENT OFFICE.

GUSTAV WALTHER, OF CREFELD, GERMANY.

## PROCESS FOR THE PRECIPITATION OF VISCOSE FOR THE PRODUCTION OF ARTIFICIAL THREADS AND OTHER STRUCTURES.

1,292,544.

Specification of Letters Patent. Patented Jan. 28, 1919.

No Drawing.

Application filed June 9, 1914. Serial No. 844,034.

To all whom it may concern:

Be it known that I, Dr. GUSTAV WALTHER, a subject of the German Emperor, residing at 16 Bissingstrasse, Crefeld, Germany, have 5 invented a new and useful Process for the Precipitation of Viscose for the Production of Artificial Threads and other Structures; and I do hereby declare the following to be a full, clear, and exact description of the 10 same.

This invention relates to the precipitation of viscose for the production of artificial threads and other structures.

The baths at present employed for this 15 purpose consist of salt and acid (German Patent No. 187947), salt and sodium bisulfate (French Patent No. 451276), glucose and sulfuric acid (British Patent No. 21405 of 1907), acids with salts and organic substances (German Patent No. 240846), or salt 20 and formic acid (French Patent No. 438718).

It is also known from the U. S. A. Patents Nos. 816404 and 849823, that threads can be 25 produced from viscose by means of sodium bisulfite solution and subsequent treatment with acids. The properties of the threads obtained in this manner however leave something to be desired.

30 According to the present invention, very good precipitation of the viscose can be effected by salts of the oxymethyl-ester of sulfuric acid, to which is attributed the following constitution:



and other aldehyde bisulfites, as well as 40 reduction products of aldehyde bisulfites like sulfoxylates



45 likewise by the similarly constituted ketone-bisulfites and also by condensation-products formed from phenols or naphthols on one hand and aldehydes and sulfites on the other, 50 such as are described on page 98 of Vol. IV of *Fortschritte der Teerfarben-Fabrikation* von Dr. P. Friedländer, vierter Teil, 1894-97, Verlag von Julius Springer, Berlin 1899.

The threads precipitate out in a homogeneous, supple, extensible and transparent state. One advantage afforded by the baths remaining perfectly clear during the precipitation, is that irregularities in the spinning can be seen at once and remedied. 60 Moreover the baths cleanse the thread being formed, brown streaks or striæ flowing from them which quickly become colorless and disappear in passing through the bath. There are no gases of decomposition formed, 65 like sulfureted hydrogen, by which the thread is easily injured, and there is likewise no separation of sulfur. The precipitation baths act extremely gently, so that the separation of the threads is very favorable. 70 Although still soluble in water, the thread exhibits great firmness and elasticity. Even after remaining for a day or more on the spool it does not lose its good qualities and withstands further treatment such as 75 twisting and winding very well.

A special advantage of the process is that the limits of maturity of the viscose in the application of the new precipitation baths are considerably wider than in the known 80 baths, which generally fail with immature or overmature viscose. It is not necessary to adhere to a definite maturity as hitherto.

The further working of the spun product into finished artificial silk can be very easily 85 accomplished, because it is scarcely possible for the undesirable sticking together or splitting of the individual threads with consequent waste of material to take place. The precipitated thread is rendered insoluble in 90 water by subsequent treatment with diluted acids, or by heating or steaming.

By means of the new process the transformation of xanthogenate-cellulose into viscose-silk can be carried out very slowly, 95 which has a favorable influence upon the properties of the thread.

The following examples may be given for the precipitation baths:—

I. 300 grams of glucose are dissolved 100 warm in 1000 grams of sodium bisulfite solution of 35-36° Baumé, and heated to 60° C. during spinning.

II. 300 grams of 40% formaldehyde are mixed with 1000 grams of sodium bisulfite 105 solution of 36° Baumé, and heated to 50° C. during spinning.

III. 186 grams of acetone are diluted with

200 grams of water, stirred up with 1000 grams of sodium bisulfite solution of 36° Baumé, and heated to 50° C. during spinning.

5 IV. 377 grams of benzaldehyde are dissolved in 1000 grams of sodium bisulfite solution of 36° Baumé, and heated to 50° C. during spinning.

V. 400 grams of rongalite are dissolved 10 in 1000 grams of water and heated to 55° C. during spinning.

The chemical composition of rongalite is:



15 VI. The product obtained from 94 grams of phenol, 250 grams of sodium sulfite and 76 grams of 40% formaldehyde, in accordance with Friedländer, Vol. IV, page 98, Example 4, is dissolved in 500 grams of water and heated to 55-60° C. during spinning.

20 According to requirements, the baths are employed either diluted or in other concentrations, and also at other temperatures than those mentioned. Moreover inorganic and 25 organic salts, such as Glauber's salt, sodium acetate and similarly acting salts, as well as

various kinds of sugar, can be added to the baths.

30 We claim:

1. A process for the precipitation of viscose for the production of artificial threads and other structures, said process consisting in introducing viscose into baths containing 35 aldehyde-bisulfites (oxymethyl-ester of sulfurous acid) and additional products; and decomposing and finishing the precipitation product.

2. A process for the precipitation of viscose for the production of artificial threads and other structures, said process consisting in introducing viscose into baths containing 40 aldehyde-bisulfites (oxymethyl-ester of sulfurous acid) and additional products with 45 the addition of substances containing sugar; and decomposing and finishing the precipitation product.

In testimony whereof, I have signed my name to this specification in the presence of 50 two subscribing witnesses.

DR. GUSTAV WALTHER.

Witnesses:

PAUL VIEES,  
HENRY AUSDFLUG.